

# UNITED STATES PATENT OFFICE.

ABRAHAM KRONSTEIN, OF KARLSRUHE, GERMANY.

## PROCESS FOR TREATING WOOD-OIL WITH OXIDIZING AGENTS.

No. 833,063.

Specification of Letters Patent.

Patented Oct. 9, 1906.

Application filed January 21, 1901. Serial No. 44,180.

*To all whom it may concern:*

Be it known that I, ABRAHAM KRONSTEIN, chemist, doctor of philosophy, and a subject of the Emperor of Austria-Hungary, residing at Karlsruhe, in the German Empire, (whose post-office address is No. 95 Kriegsstrasse, Karlsruhe, Germany,) have invented a certain new and useful Process for Treating Wood-Oil with Oxidizing Agents, of which the following is a specification.

This invention has reference to a process for preventing the coagulation of wood-oil (tung-oil) during the action thereon of oxidizing agents, such as dioxid of lead, minium, chromic salts, atmospheric air, and similar agents that split off or transmit free oxygen or oxidizing oxygen-yielding driers as used in the manufacture of varnishes. This so-called "Chinese" wood-oil is the oil expressed from the berries of the tree generally known as "*Aleurites cordata*" or "*Elæococca vernicia*" and sometimes also called "tung-oil" in the trade. For the sake of brevity I shall refer to it in the following specification and claims simply as "wood-oil" it being understood that only the oil referred to is meant. The property of wood-oil of coagulating and forming a "curd," so to speak, upon the action of oxidizing agents or driers as employed in the manufacture of varnishes, japs, and the like has heretofore been a great drawback in the use of wood-oil in the arts. This inconvenience may be avoided by previously mixing the wood-oil in suitable proportions with such drying-oils, resins, or solvents, which prevent the polymerization of wood-oil by producing a dissociating action upon its molecule. Such mixtures of wood-oil or tung-oil with other organic varnish-forming substances, and in particular with drying-oils or resins or substances having a similar chemical constitution, where the quantity of wood-oil or tung-oil is sufficiently below the total amount of the other varnish-forming organic constituents of the mixture to enable them to remain liquid upon exposure to high heat will also refuse to yield a curd when they are treated with oxidizing agents, such as chromates or artificial oxidizing oxygen-yielding driers, such as lead or manganese compounds, and, on the other hand, such mixtures containing so large a percentage of wood-oil that prolonged heating will convert them into a solid mass may also be treated with oxidizing oxygen-yield-

ing driers, chromates, or the like in the manufacture of varnishes, japs, and for other purposes without fear of forming the undesired jelly or curd if the heating is interrupted and the addition of the oxidizing agent is made before solidification can set in, resins, drying-oils, or the like being added along with or immediately after the addition of oxidizing agents. In order to be able to treat the solidified compounds which are obtained by heating mixtures of an excess of wood-oil with other drying-oils or equivalent substances with oxidizing agents or oxidizing oxygen-yielding driers, the said solid bodies are subjected to a process of remelting with drying-oils, resins, or equivalent substances. They are thereby converted into a viscous oil which may be treated with oxidizing agents or artificial oxidizing oxygen-yielding driers for the manufacture of varnishes and the like without fear of curdling. I am thus enabled to convert both the original untreated wood-oil as well as the wood-oil which has been subjected to a thickening or solidifying process into a modification which when treated with oxidizing agents will not gelatinize. The nature of the oxidizing agent or oxidizing oxygen-yielding drier used is perfectly immaterial.

As regards the mixtures themselves, drying-oils will be used in quantities of more than fifty per cent. of the mixture. If resin is used, the amount of resin to be added to the wood-oil in order to produce the desired effect of preventing gelatinization on treatment with oxidizing agents or oxidizing oxygen-yielding driers seems to depend upon the amount of partly-volatile resin-oil constituents in the resin, while of rosin only about thirty per cent. any more need to be added to the mixture. More than fifty per cent. is necessary with dammar, Venetian turpentine, melted amber, and gutta-percha. Gum-copal requires a still greater percentage—that is to say, more than seventy per cent. If mixtures of different kinds of resin or with drying-oils are used, the quantities of these admixtures required for preventing gelatinization upon the addition of oxidizing agents will of course be different. The same effect is produced by an addition of solvents such as oil of turpentine, benzol, camphor-oil, and the like if the admixtures amount to more than twenty per cent. Such solvents will prevent gelatinization during the treat-

ment with oxidizing oxygen-yielding driers or with oxidizing agent of wood-oil, as well as of mixtures of wood-oil, which otherwise when heated alone yield a solid body which is insoluble in the ordinary solvents.

In carrying out my invention I may, as aforesaid, make use of oil mixtures which under ordinary circumstances yield insoluble products by prolonged heating, and I may then proceed as follows: Wood-oil or such mixtures thereof as otherwise solidify during the heating process of suitable duration are rapidly heated up to a temperature of from about 270° to 280° centigrade, no solidification taking place at this rapid heating. I then add rapidly any desired oxidizing agent, in small quantities at a time, which dissolves in the oil mixture. The heating process is then interrupted by closing a damper or otherwise and the mixture cooled down below the boiling-point of the solvent which it is desired to add. After this addition has been made the thus-diluted mixture is then boiled in a vessel provided with a condenser, the volatilized portions condensing and dropping back into the mixture.

I may mention the following examples of carrying my invention into effect:

Example 1: One hundred pounds wood-oil and one hundred and twenty pounds linseed-oil are treated as usually with oxid of lead, minium, borate of manganese, air, or other oxidizing agents.

Example 2: One hundred pounds wood-oil which have been previously thickened by heating are dissolved in one hundred and twenty pounds linseed-oil and are then treated as shown with reference to Example 1.

Example 3: One hundred pounds wood-oil which have been rendered insoluble by prolonged heating are melted, diluted with one hundred and twenty pounds of linseed-oil, and are then treated in like manner as in Example 1.

Example 4: One hundred pounds of the oil produced by remelting the solid body obtained from a mixture of one hundred and twenty pounds wood-oil and eighty pounds linseed-oil by prolonged heating are mixed with sixty pounds linseed-oil and are then treated as in Example 1.

Example 5: One hundred and twenty pounds of dammar resin are dissolved in one hundred pounds wood-oil and treated with oxidizing agents in the usual manner.

Example 6: Two hundred pounds of a mixture of one hundred and twenty pounds of wood-oil and eighty pounds dammar resin are heated, and to this mixture I add sixty pounds more of dammar before solidification can set in or in case the mixture should have become already solidified after remelting the solid body obtained, and I then treat with oxidizing agents in the ordinary way.

Example 7: In place of the resin I use

sixty pounds of linseed-oil as an addition to the mixture of wood-oil and dammar described in Example 6.

Example 8: One hundred and forty pounds of wood-oil are heated to about 270° centigrade and are then mixed with from two to three per cent. of oxid of lead. On stirring the mixture the lead oxid will dissolve therein. The mixture is then cooled down to about 120° centigrade and mixed with sixty pounds of oil of turpentine, and the whole mass is finally boiled for from two to three hours in a vessel to which is connected a reflux condenser.

What I claim, and desire to secure by Letters Patent of the United States, is—

1. The process of preventing the coagulation of wood-oil, obtained from *Aleurites* plants, occurring upon the treatment of said oil with oxidizing agents which consists in mixing and heating said oil, substantially as described with a quantity of resin and vegetable drying-oils in excess of the amount necessary for changing the mixture into a solid, insoluble gum, and with oxidizing, oxygen-yielding driers, substantially as described.

2. The process of preventing the coagulation of wood-oil, obtained from *Aleurites* plants, occurring upon the treatment of said oils and of mixtures of the same with vegetable drying-oils, resins and solvents, with oxidizing or oxygen-yielding agents, which process consists in heating the mixtures of wood-oil with other drying-oils coagulated by heating with an excess of other drying-oils but wood-oil, until liquefaction takes place.

3. The process of preventing the coagulation of wood-oil, obtained from *Aleurites* plants, occurring upon the treatment of said oils and of mixtures of the same with vegetable drying-oils, resins and solvents, with oxidizing or oxygen-yielding agents, which process consists in heating the mixtures of wood-oil with resins coagulated by heating with an excess of other drying-oils but wood-oil, until liquefaction takes place.

4. The process of preventing the coagulation of wood-oil, obtained from *Aleurites* plants, occurring upon the treatment of said oils and of mixtures of the same with vegetable drying-oils, resins and solvents, with oxidizing or oxygen-yielding agents, which process consists in heating the mixtures of wood-oil with solvents coagulated by heating with an excess of other drying-oils but wood-oil, until liquefaction takes place.

5. The process of preventing the coagulation of wood-oil, obtained from *Aleurites* plants, occurring upon the treatment of said oils and of mixtures of the same with vegetable drying-oils, resins and solvents, with oxidizing or oxygen-yielding agents, which process consists in heating the mixtures of wood-oil with other drying-oils coagulated

by heating with resins and with oxidizing, oxygen-yielding agents, until liquefaction takes place.

6. The process of preventing the coagulation of wood-oil, obtained from *Aleurites* plants, occurring upon the treatment of said oils and of mixtures of the same with vegetable drying-oils, resins and solvents, with oxidizing or oxygen-yielding agents, which 10 process consists in heating the mixtures of wood-oil with resins coagulated by heating with resins and with oxidizing, oxygen-yielding agents, until liquefaction takes place.

7. The process of preventing the coagulation of wood-oil, obtained from *Aleurites* plants, occurring upon the treatment of said oils and of mixtures of the same with vegetable drying-oils, resins and solvents, with oxidizing or oxygen-yielding agents, which 15 process consists in heating the mixtures of wood-oil with solvents coagulated by heating with resins and with oxidizing, oxygen-yielding agents, until liquefaction takes place.

8. The process of preventing the coagulation of wood-oil, obtained from *Aleurites* plants in the manufacture of varnishes, japs and the like which consists in first heating a mixture of wood-oil and varnish-form-

ing organic constituents until solidification sets in, then adding a new quantity of organic varnish-forming constituents to the solidified mass and rapidly heating the same until liquefaction takes place, and then mixing oxidizing agents or driers with the liquefied mixture.

9. The process of preventing the coagulation of wood-oil, obtained from *Aleurites* plants in the manufacture of varnishes, japs and the like which consists in mixing wood-oil or tung-oil with resins, the amount 30 of resin being governed by its percentage of volatile oil, then combining the constituents of said mixture by heating the same, then adding oxidizing agents or driers to the resultant liquid while still in hot condition, 35 then cooling the mixture, then adding a solvent, and finally boiling the mixture and solvent, substantially as described.

In witness whereof I have hereunto signed my name in the presence of two subscribing 40 witnesses.

ABRAHAM KRONSTEIN.

Witnesses:

WOLDEMAR HAUPT,  
HENRY HASPER.